

No. 823,345.

PATENTED JUNE 12, 1906.

T. H. MATHIAS.  
ART OF ROLLING METAL PLATES.  
APPLICATION FILED SEPT. 16, 1904.

2 SHEETS—SHEET 1.



FIG. 1



FIG. 2



FIG. 3

WITNESSES:

A. J. A. B. McCauley.  
Loretto O'Connell

INVENTOR  
J. H. Mathias,  
BY  
Geo. H. Parmelee,  
his ATTORNEY.

No. 823,345.

PATENTED JUNE 12, 1906

T. H. MATHIAS.  
ART OF ROLLING METAL PLATES.  
APPLICATION FILED SEPT. 18, 1904.

2 SHEETS—SHEET 2.



FIG. 4



FIG. 5



FIG. 6

WITNESSES:

A. A. B. M. Bailey  
Loretta O'Connell

J. H. Mathias,  
INVENTOR  
BY  
Geo. H. Parmelee,  
his ATTORNEY.

# UNITED STATES PATENT OFFICE.

THOMAS H. MATHIAS, OF CHICAGO, ILLINOIS, ASSIGNOR TO ILLINOIS STEEL COMPANY, A CORPORATION OF ILLINOIS.

## ART OF ROLLING METAL PLATES.

No. 823,345.

Specification of Letters Patent.

Patented June 12, 1906.

Application filed September 16, 1904. Serial No. 224,857.

*To all whom it may concern:*

Be it known that I, THOMAS H. MATHIAS, of Chicago, in the county of Cook and State of Illinois, have invented a new and useful Improvement in the Art of Rolling Metal Plates, of which the following is a full, clear, and exact description, reference being had to the accompanying drawings, which form a part of this specification.

It is the usual practice in the manufacture of rolled plates—such as ship-plates, tank-plates, boiler-plates, and the like—to first roll the ingots into slabs of rectangular cross-section, these slabs being subsequently reheated and transferred to the plate-mill, where they are rolled into plates of the desired dimensions. In rolling plates of considerable width, such as those fifty inches wide and upward, the plates on leaving the rolls show a fish-tail shape to such an extent that they may vary from twenty to thirty inches in length between the center and the ends, thereby causing a considerable percentage of loss in trimmings or "plate scrap." This fish-tailing is due to the spring in the rolls, which causes the plate to be thinner at the sides than at the middle and causes a displacement or squeezing of the metal at the lateral portions of the plate toward its ends, the result being that the plate becomes longer at the sides than at the middle. The fish-tail ends of the plate are also hard on the rolls, as they become chilled and hard.

My invention is designed to provide an improved method of rolling plates which will prevent the formation of these fish-tail ends, thereby reducing very largely the percentage of plate scrap and increasing the plate percentage. My new method by preventing the formation of fish-tails also greatly relieves the rolls by providing better plate ends upon which they can get a square bite across the entire width of the plate. These objects I accomplish in the following manner.

In the first place I depart from the usual practice of employing rectangular slabs of substantially uniform thickness throughout and instead I roll a slab of symmetrical cross-section in which the lateral portions are thinner than the central portion throughout the length of the slab. I then reheat this slab and transfer it to the plate-mill having plain

cylindric rolls, where it is first rolled in the same direction that it passed through the rolls of the slabbing-mill. The result of this 55 rolling is to cause the thicker metal at the longitudinal central portion of the slab to flow toward the ends of the plate, so that after being passed several times through the rolls in this direction the ends of the plate are of 60 convex form—that is to say, the plate is longer on its middle line than at its lateral edges. The plate is now turned and passed a number of times through the rolls in a direction at right angles to the direction in 65 which the slab was rolled. This operation gives the plate the requisite width, but still leaves the plate longer along its middle line than at the edges, taking such middle line through the plate in a direction parallel to 70 that in which the slab was rolled. This cross-rolling also very considerably increases the tensile strength and elastic limit of the finished plate. The plate is now again turned and rolled in the same direction as at first to 75 the proper thickness or gage. The effect of this last rolling is to cause the metal at the lateral portions of the plate to flow in the direction of the rolling faster than the metal at the central portion, due to the spring of the 80 rolls, while the metal at the central portion tends to be squeezed or displaced toward the lateral portions, the final result being the formation of a plate whose ends are approximately straight and in which the waste to be 85 trimmed is reduced to a minimum.

In the accompanying drawings, Figure 1 is a view showing the character of rolls employed in the slabbing-mill for the purpose of rolling the slabs; Fig. 2, a perspective view 90 of one of the slabs; Fig. 3, a cross-section of the same; Fig. 4, a plan view showing approximately the shape of the plate after the first step in rolling; Fig. 5, a similar view showing the approximate form of the plate 95 after the second rolling, and Fig. 6 a similar view of the plate as it finally leaves the rolls.

The slab A leaves the finishing-pass b of the slabbing-rolls B in the form shown in Figs. 2 and 3—that is to say, with its lateral 100 portions a thinner than its central portion—the reduction in thickness being at both the upper and the lower surfaces of the slab, which is preferably of symmetrical cross-section.

The reduction from the greater to the lesser thickness is a more or less graduated one, as shown at  $a'$ , and the angles at  $a^2$  are preferably slightly rounded in order to ease the rolls. The extent of the difference in thickness between the central and the lateral portions of the slab will naturally vary somewhat with the dimensions of the slab and the dimensions of the plates to be rolled. In a slab of thirty-six inches in width, which under the old practice would be of a uniform thickness of five inches, I find it advisable to increase the thickness to about five and one-half inches at the central portion for somewhat more than one-half the total width of the slab and then to gradually taper down to a thickness of five inches, which is held to its lateral edges. These figures and the precise section illustrated in the drawings are, however, merely illustrative and may be considerably varied, the essential feature being in every case to provide an excess of metal at the central over the lateral portions of the slab sufficient to take care of the displacement described, and this is a matter which the experienced roller can readily determine by observation. I do not, therefore, limit myself to the use of a slab of the particular section shown and described.

Having thus described my invention, what I claim as new, and desire to secure by Letters Patent, is—

1. The art or method of rolling metal plates, which consists in forming a slab having an excess of metal at its longitudinal central portion, then rolling said slab first in the direction of its length and second, at right angles to such direction, and finally rolling the shape produced by the preceding steps in the same direction as at first, the last two rolling operations being with plain cylindrical rolls.

2. The art or method of rolling metal plates, which consists in first forming a slab having an excess of metal at its longitudinal central portion but of the same cross-section throughout its length, then rerolling said slab first in the direction of its length, then at right angles to the first rerolling, and finally, in the same direction as at first, the first and second rerolling operations being with plain cylindrical rolls, for the purposes described.

In testimony whereof I have affixed my signature in presence of two witnesses.

THOMAS H. MATHIAS.

Witnesses:

JOHN R. EMERSON,  
GUY ROCHE JOHNSON.